

# UNITED STATES PATENT OFFICE.

JOSEF RUDOLF, OF GERA, GERMANY.

## PROCESS OF WATERPROOFING AND FINISHING TEXTILE MATERIAL.

SPECIFICATION forming part of Letters Patent No. 653,701, dated July 17, 1900.

Application filed March 26, 1898. Serial No. 675,283. (No specimens.)

To all whom it may concern:

Be it known that I, JOSEF RUDOLF, a subject of the Emperor of Germany, and a resident of 31 Thalstrasse, Gera, in the Principality of Reuss, in the Empire of Germany, have invented a new and useful Improved Process of Waterproofing and Finishing Textile Material, of which the following is a specification.

10 Hitherto paraffin, stearates, wax, and the like solid substances have been employed in the following way for rendering fabrics and the like waterproof: First, by causing a hot roller to rotate against the said solid substances and then conveying the goods against the said roller, or, secondly, by dissolving these substances in benzole, benzin, or the like and saturating the goods with such solution. The first-named process has the drawback that it is very difficult to effect an even distribution of coating. The second is too expensive in consequence of the solvents employed.

This invention has for its object an improved process for rendering textile materials, wood substances, and the like waterproof and for protecting them against spotting and moths. The improved process is characterized by the use of substances insoluble in water, such, for instance, as solid hydrocarbon, in the form of paraffin or ozocerite, stearin, palmitin, and their metallic compounds, (such as stearate, palmitate, and resinate of aluminium, calcium, zinc, and the

like compounds,) vegetable wax, and beeswax, resins, and the like being melted and emulsified or mixed in liquid condition in hot water by suitable means in such a way that the mixture approximates to a solution, the articles, materials, or goods being then coated or otherwise saturated with a thin film of this mixture, while the latter is applied at such a high temperature that the water or fluid evaporates and the waterproofing or finishing substances are melted into the goods.

The above-named substances can be used either singly or in mixture in the following proportions: paraffin, one part; aluminium stearate, half a part; ozocerite, two parts, and wax one part.

Having thus described my invention, the following is what I claim as new therein and desire to secure by Letters Patent:

The improved process for waterproofing and finishing textile materials, which consists in reducing the waterproofing material to a molten condition, next making an emulsion of the same in hot water, and then applying the said emulsion while maintained at a high temperature, to the material to be waterproofed.

The foregoing specification is signed at Gera, Reuss, German Empire, this 2d day of February, 1898.

JOSEF RUDOLF.

In presence of—

A. BRÄUTIGAM,  
G. MÜLLER.